

Dec. 2, 1969

S. O. DORST

3,481,779

FILM RESISTOR AND METHOD

Filed July 22, 1966

*Fig.1.*

*Depositing A Coat  
On A Refractory Body*

*Devitrifying The Surface  
Of The Coated Body*

*Cleaning The Treated  
Surface*

*Depositing A Film On  
The Cleaned Surface*

*Fig.2.*



*Devitrified and Etched Surface*

## 1

3,481,779

### FILM RESISTOR AND METHOD

Stanley O. Dorst, Nashua, N.H., assignor to Sprague Electric Company, North Adams, Mass., a corporation of Massachusetts

Filed July 22, 1966, Ser. No. 567,053

Int. Cl. B44d 1/20, 1/02; C23b 5/02

U.S. Cl. 117—213

9 Claims

### ABSTRACT OF THE DISCLOSURE

A resistive film is provided on a devitrified and etched surface of a refractory material having glassy and crystalline phases. The surface is prepared by the deposition of a resistive coating on the surface and then burning off the coating.

The present invention relates to film resistors and more particularly to an improved surface for the bodies carrying resistance films in electrical resistors and a process for producing the improved surface.

Metal film resistors are made up by the application of a thin film of metal to a supporting surface of dielectric material. The metal film is a conductive layer having desired ohmic characteristics. The substances used for supporting the resistive films include, for example, electrical porcelain or alumina having deposited thereon suitable compositions in a film; such as, for example, Nichrome to provide desired ohmic values.

The metal film is deposited on the surface by a procedure providing uniform ohmic characteristics across the resistive film, such as by evaporation onto the supporting surface. The metal film may be deposited on refractory material having glassy and crystal phases where materials are required which retain high structural strength at elevated temperatures and have good dielectric properties.

It is desirable to provide superior resistance characteristics in the films of the resistors. An increase in ohmic value is desirable without the sacrifice of electrical characteristics in the resultant resistor unit. An increase in ohmic value permits a greater resistance per unit volume. While the increase of apparent surface area of the supporting dielectric material is desirable and tends toward increased ohmic value, previously the apparent increase of surface area has been susceptible to change during subsequent processing of the unit resulting in diminution of the resistive properties in the final structure.

It is an object of this invention to provide a film resistor having superior resistive and electrical properties.

It is another object of this invention to provide an improved refractory body having glassy and crystal phases for a resistive film.

It is a further object of this invention to produce a metal film resistor having a higher resistance per unit volume.

Another object of this invention is to provide a process for making a thin film electrical resistor with good electrical characteristics on a ceramic body having glassy and crystal phases.

Still another object of this invention is to provide a process for preparing micro-crystalline surfaces for resistive films.

It is a still further object of this invention to provide a simple and effective process for preparing a large number of film resistors in a single manufacturing procedure.

In general, this invention involves a resistive film on a devitrified and etched surface of a refractory material having glassy and crystal phases providing a film resistor having improved ohmic values. The resistive film, such as, Nichrome, is applied to the refractory surface after

## 2

preparation of the surface by the deposition of carbon and burning the carbon coat off, ultrasonic cleaning the treated surface and finally metallizing the prepared bodies, preferably while rotating.

In a drawing which illustrates this invention, FIGURE 1 is a flow sheet of the process, and FIGURE 2 is a cross-section of the resistor with identification of the devitrified and etched surface.

The surface of the essentially noncrystalline glassy phase is modified to an apparent crystalline state by devitrification while the crystal phase of the refractory material is etched at the grain boundaries at the surface. In the vitreous state the solid glassy phase is essentially non-crystalline and may be thought of as a disordered amorphous solid with a glassy surface. The process of this invention devitrifies this surface to a state resembling the crystalline state.

More particularly, a ceramic core having glassy and crystal phases has the surface modified by a thermal devitrification and etch process. The surface is first modified so that the glassy surface is devitrified and then the surface is cleaned to remove material. The surface is a refractory dielectric material then ready for the application of the metal film resistance element by a suitable procedure.

A preferred processing of the refractory involves coating the refractory surface in a closed system to provide a coating of devitrified material on the surface. After coating, the coated refractory body is cooled and then immediately heated in the closed reaction chamber in the presence of oxygen. The treated structures are then cleaned to remove material loosened in the process. The cleaning leaves the surface ready to receive the deposition of a resistive film. The surface of the glassy phase is apparently devitrified.

More specifically, this invention provides the superior resistance element on a ceramic core by first rotating the cores in large batches in a closed reaction chamber in the closed system while suitably coating the core surfaces with a carbon coating, such as by pyrolysis of a hydrocarbon gas in an inert carrier in the closed chamber. The temperature in the reaction chamber is then reduced under the passage of inert gas but otherwise closed. As soon as the cooling is complete, the carbon coat is burned off the surfaces in a flow of oxygen-containing gas by raising the closed chamber temperature. Next the treated cores are ultrasonically cleaned to remove loose material after which a resistive film is applied to the treated cores by metallization while rotating the chamber containing the cores.

Apparatus for the practice of this invention is primarily a reaction chamber in a closed system which may for example, be a quartz bottle and in which the cores to be processed are placed. Conduits open into the chamber for admitting active and inert gases and valves are provided for sealing the chamber.

As an example of the process of surface improvement, reference is made to the production of Nichrome film resistors on ceramic cores. The cores are placed in a rotating reaction chamber in a closed system and heated while hydrocarbon gas in an inert carrier such as nitrogen is introduced and striking the hot cores and pyrolyzes to deposit a carbon coating on the core surface. Upon completion of the coating, the hydrocarbon gas is turned off and cool oxygen-free nitrogen continues to flow at temperatures to gradually cool the cores in the closed chamber. Then, while the chamber remains closed, the carbon coated rotating cores are subjected to reheating at a temperature in the range of 1500° to 1900° F. in a passage of oxygen-containing gas through the system for about four hours to burn off the carbon. It has been dis-

covered that a superior improvement in ohmic value is achieved in holding the carbon coated surfaces in the chamber atmosphere standing sealed from the ambient atmosphere and proceeding with the burn-off as soon as the cooling is complete.

The cores are ultrasonically cleaned. This completes the preparation of the surface for the reception of the metal film.

The prepared cores are then preferably strung on rods which are mounted so that the carriage rotates on its axis revolving the cores around a common axis and are mounted so that they revolve while a Nichrome filament centrally located is heated to a vaporization temperature and is deposited on the moving cores.

While burning off the carbon coating provides an increase in ohmic value, a particularly desirable increase can be obtained by burning off the carbon coating with continuous rotation of the containers in which the bodies are held.

Without limiting this invention, the following examples are given to illustrate the preferred mode of operation.

#### EXAMPLE I

Ceramic cores for metal film resistors are placed in a closed quartz bottle and heated. A methane gas mixture in nitrogen is introduced into the quartz bottle through a closed system and passed over the heated cores. Pyrolysis of the methane gas at the pre-heated core surfaces deposits a carbon coating on the core surfaces. The quartz bottles are continuously rotating during the passage of the methane gas mixture the pyrolysis and carbon coating. After the deposition of carbon completely covers the tumbled cores with a carbon coating, the methane gas is turned off and a cooled oxygen-free nitrogen gas flows into the quartz bottle and cools the cores gradually in an atmosphere sealed from the atmosphere. The cooling off under the nitrogen gas flow is continued for 45 minutes. The closed quartz bottles are still rotated while oxygen is passed through the system and the cores are reheated to a temperature of about 1840° F. for about four hours and the carbon coating is burned off. The surface in the glassy phase is devitrified and the surface in the crystal phase is etched. The bottles are then opened and the cores are then ultrasonically cleaned after which the cores are strung on rods mounted in a rotating carriage which is revolved around an axis. The carriage is rotated on its axis to revolve the cores while each core rotates on its own axis. A Nichrome filament centrally located in the rotating carriage is vaporized by heating to a vaporization temperature and then a Nichrome composition is deposited on the moving cores which are maintained at a lower temperature to receive a deposition of the Nichrome film.

The gain in ohmic value of the resistive film which is produced is several times the ohmic value of a Nichrome resistive film on a similar untreated ceramic core.

#### EXAMPLE II

The method of Example I is utilized to produce a carbon coat on the surface of ceramic cores, and the cores sealed in the quartz bottles against the introduction of oxygen-containing gas are cooled under a flow of nitrogen gas for 45 minutes. The sealed quartz bottles are still rotated while the carbon coated cores are reheated to a temperature of about 1500° F. for about four hours. The carbon coating is burned off leaving the core surface devitrified in the glassy phase and etched in the crystal phase. The cores are then ultrasonically cleaned and coated with a Nichrome composition utilizing the method of Example I. The resistive film thus prepared has a gain in ohmic value of several times that of a resistive film applied to an untreated ceramic core.

#### EXAMPLE III

The method of Example I is utilized to produce a

resistive Nichrome film on a batch of 1,000 cores in a single container. A greater increase in ohmic value is obtained in the resistive film thus produced.

It will be understood that the details of procedure above set forth may vary widely within the skill of those engaged in this art. The following additional details will assist in the understanding and application of the invention.

Continuous rotation is preferred. Although the tumbling of the cores during processing may be reduced to a periodic 180° rotation of the container at intervals of several minutes, the gain in ohmic value is substantially decreased as a consequence.

Among other advantages, the process of this invention provides a metal film resistor having superior resistive properties with adequate or superior electrical characteristics; such as, a low noise factor.

This invention applies to metal film resistors, such as, high precision, high stability metal film resistors over a range of resistances. This development, however, is of particular interest in application to the higher resistance values in the range of standard resistance values, as for example, resistances in the megohm ranges. The resistors of this invention have a satisfactory temperature coefficient of resistance, such as for example, around 75 p.p.m./° C. through a wide temperature range. The novel articles embodying useful aspects of this invention include a metal film resistor incorporating a high resistance value on a small ceramic core. The practical effect of the increased ohmic value is better component density. At the same time other important properties and characteristics of high precision, high stability metal film resistors are maintained.

It will be understood that the reference to the production of Nichrome film resistors on electrical porcelain cores is by way of example of the process of surface improvement. Further modifications are within the spirit of this invention. For example, cooling of the carbon coated cores under the passage of oxygen-free nitrogen for 45 minutes is preferred, but lesser periods of cooling in the specified procedure provides substantial increases in ohmic value.

What is claimed is:

1. A method of producing a film resistance element on the surface of a refractory body having both a glassy phase and a crystal phase comprising the steps of at least:

- depositing a resistive coating on the surface of the glassy phase of the body;
- burning off the coating to devitrify the surface of the glassy phase;
- cleaning the article surface;
- depositing a resistor film on the clean surface including the glassy phase.

2. The method of improving the ohmic value achieved with a resistive film on a surface area of a refractory body having both a glassy phase and a crystal phase which comprises providing said refractory bodies, preheating the bodies to a temperature in excess of a hydrocarbon pyrolyzing temperature, exposing the preheated bodies to a hydrocarbon gas mixture to pyrolyze the hydrocarbon and cause a carbon layer to deposit on the surfaces of the bodies, cooling the coated bodies, heating the coated bodies in oxygen-containing gas to burn off the carbon, cleaning the treated surfaces after carbon burn off, and depositing a resistor film on the clean surface.

3. The method of improving a resistive film as set forth in claim 2 in which the carbon coated body is heated to a temperature of at least 1500° F. and the carbon is burned off.

4. The method of improving a resistive film as set forth in claim 2 which is accompanied by etching the surface of the crystal phase of said bodies.

5. The method of improving a resistive film as set forth in claim 2 in which the carbon burn off is con-

ducted without exposing the bodies to ambient air following the deposition of the carbon layer.

6. A metal film resistor including a non-conducting substrate having a glassy phase and a crystal phase, the surface of the glassy phase being devitrified and the surface of the crystal phase being etched and a thin film resistance element on said substrate having stable ohmic characteristics.

7. The metal film resistor of claim 6 wherein the substrate consists of a ceramic.

8. The metal film resistor of claim 6 wherein the devitrified surface of the glassy phase is micro-crystalline.

9. The metal film resistor of claim 6 wherein the resistance element consists of Nichrome.

#### References Cited

##### UNITED STATES PATENTS

3,266,912 8/1966 Murphy ----- 106—1

WILLIAM L. JARVIS, Primary Examiner

10 U.S. Cl. X.R.

29—620; 65—30, 33; 117—227, 107.1, 54